

March 1, 1949.

F. HUTCHINSON

2,463,388

CONTAMINATION RESISTING HAT FOR MAGNETRONS

Filed Jan. 3, 1946

FIG. 1



FIG. 2



INVENTOR  
FRANKLIN HUTCHINSON  
BY

*William D. Hall*  
ATTORNEY

## UNITED STATES PATENT OFFICE

2,463,388

CONTAMINATION RESISTING HAT FOR  
MAGNETRONS

Franklin Hutchinson, New Haven, Conn., assignor, by mesne assignments, to the United States of America as represented by the Secretary of War

Application January 3, 1946, Serial No. 638,884

3 Claims. (Cl. 250—27.5)

1

My invention relates to thermionic tube apparatus and more particularly to the emitting members of such tubes.

In thermionic apparatus of the magnetron type, there is provided an anode, an emitting cathode and a shield or "hat" member positioned adjacent the cathode for the purpose of constricting the path in which the electrons from the cathode may travel. In those magnetrons whose cathode hats normally attain a temperature of around 700° C. or higher, certain phenomena, usually referred to as "leakage," are sometimes noted during the performance of the tube. These phenomena are believed to be due in part to the emission of electrons from the hat possibly owing to their becoming coated in some fashion with oxide coating material from the emitting surface of the cathode. Accordingly, it is one of the objects of my invention to provide a device in which this effect is minimized.

In the prior art to which this invention belongs, attempts have been made to prevent emission from the shield or hat by coating the hat with materials such as tungsten powder, zirconium and some other materials which are supposed to be poor bases for oxide materials used in cathodes and which evaporates from the cathode and deposits on the shield. This has not proven altogether satisfactory because, while the device will work in a desirable fashion for a limited period of time, after a while noticeable leakage occurs possibly due to the inequality in expansion between the tungsten or zirconium and the nickel base with which it is usually used. Again the zirconium presents difficulties in coating and considerable labor is involved in preparing the shield member. Accordingly it is an object of the present invention to provide a more satisfactory and desirable form of shield or hat arrangement which eliminates the use of poison materials on the hat by making the hat itself of a material which in itself is a poor base for oxides of which the cathodes normally are formed.

It is a further object of my invention to provide a shield or hat arrangement for use with the cathode in the magnetron which will be highly satisfactory, simple in nature and easy to manufacture.

It has been found that substantially pure iron having a very thin film of barium and/or strontium oxide evaporated onto it such as would occur in the operation of a magnetron for instance, has a very poor electron emission characteristic. Therefore by making the hat or shield of this

2

material, the aims and objects of the invention are accomplished. Relative emission characteristics will be described hereinafter with respect to the description of Fig. 3. My invention will best be understood by reference to the drawings in which:

Fig. 1 is a partial top view of a vane type of magnetron showing the principle of my invention;

10 Fig. 2 is a cross-sectional view along line 2—2 of Fig. 1;

Referring to Fig. 1, there is shown a partial top view of a vane type of magnetron constructed in accordance with my invention. In this view 15 the position of a portion of the vanes relative to the cathode is illustrated. The cathode 10 having the hat members 11 at the ends thereof is located at the center of the apparatus, and the anode members 12 are radially disposed thereabout and are spaced at equal distance around the cathode. It will be appreciated that this is merely an illustrative arrangement and no attempt has been made to show either the proper number or the desirable number of vanes that 20 might be used in the magnetron.

Referring to Fig. 2, there is shown a relative arrangement of the cathode 10 having the hat members 11 constructed of Svea iron with respect to the anode members 12. This is a partial 25 view on a cutting plane taken along a line of sight 2—2 of Fig. 1. The object of this view is merely to illustrate the relative position of the upper and lower edges of the vane and the hat members on the cathode. It will further be appreciated that this is for illustrative purposes only and that the arrangement could be equally well applied to the so-called resonant cavity type of magnetron as well as other types.

30 Sleeves of typical cathode shield material were 40 tested for electron emission under typical conditions met with in service after having been prepared in a manner also typical of the conditions met with in service. These test sleeves were prepared by being heated and then having evaporated onto them an amount of electron emitting oxide coating equivalent to the amount evaporated onto a shield from a cathode operating at 350° centigrade for hundreds of hours.

The D.-C. emission from the sleeve at 400 volts 45 50 plate potential as a function of temperature was taken over a range of temperatures in which the emission was stable. The following emission was noted:

Where the test sleeve was comprised of zirconium powder in a nitrocellulose binder and op-

erated on grade "A" nickel where the sleeve had been heated up to 1000° centigrade and then held at approximately 600° centigrade during evaporation of the oxide cathode, the emission of 800° Centigrade operating temperature of the sleeve was from 20 to 40 milliamperes per square centimeter with 400 volts D.-C. potential on the plate of the tube. The data is not available on its pulsed emission having a pulse length of 1 microsecond and pulsed 60 cycles per second at 5 kilovolts anode potential.

Grade "A" nickel 3 millimeter tubing from Superior Tube Company (1941), when comprising a sleeve which has been flashed at substantially 1000° Centigrade and then held at substantially 800° Centigrade during evaporation of the oxide cathode, showed a D.-C. emission of 5 to 10 milliamperes per square centimeter with 400 volts anode potential in the tube and showed a pulsed emission of .1 amperes per square centimeter at 1000° Centigrade operating temperature where the pulses were 1 microsecond in length and the pulse rate was 60 per second with 5 kilovolts anode potential.

Svea metal tubes from .005 inch sheet metal manufactured by the Swedish Iron Corporation of America and flashed at substantially 1000° Centigrade and then held at substantially 600° Centigrade during evaporation of the oxide cathode showed zero emission at 800° operating temperature and 400 volts D.-C. potential on the anode of the tube. Its pulsed emission under the same conditions as the grade "A" nickel was too low to observe.

While the preferred embodiment of this invention has been set forth hereinbefore, it will be appreciated that there may be deviations therefrom which will fall within the spirit of the invention and accordingly I claim such deviations which fall fairly within the spirit and scope of the hereinafter appended claims.

What is claimed is:

1. A magnetron cathode having no end leakage comprising a cylindrical cathode having an electron emitting coating on its cylindrical surface and shields enclosing the ends of said cylindrical cathode, the said shields being made of iron.
- 10 2. A magnetron cathode having no end leakage comprising a cylindrical cathode with a cylindrical electron emitting surface and shield hats made of iron enclosing the ends of said cathode.
- 15 3. A cathode for a high frequency thermionic tube having no end leakage comprising a cathode having electron emitting longitudinal surfaces and end surfaces, and shield hats made of iron fitted over said end surfaces.

FRANKLIN HUTCHINSON.

#### REFERENCES CITED

The following references are of record in the file of this patent:

#### UNITED STATES PATENTS

| Number    | Name        | Date          |
|-----------|-------------|---------------|
| 1,886,705 | Lucian      | Nov. 8, 1932  |
| 2,208,406 | Benedict    | July 16, 1940 |
| 2,418,117 | Hale et al. | Apr. 1, 1947  |